

May 4, 1937.

S. L. INGERSOLL

2,079,213

METHOD OF MAKING LAMINATED METAL

Filed Nov. 23, 1934

2 Sheets-Sheet 1



May 4, 1937.

S. L. INGERSOLL

2,079,213

METHOD OF MAKING LAMINATED METAL

Filed Nov. 23, 1934

2 Sheets-Sheet 2



## UNITED STATES PATENT OFFICE

2,079,213

## METHOD OF MAKING LAMINATED METAL

Stephen L. Ingersoll, Chicago, Ill., assignor, by  
mesne assignments, to Borg-Warner Corporation,  
Chicago, Ill., a corporation of Illinois

Application November 23, 1934, Serial No. 754,462

9 Claims. (Cl. 29—189)

This invention relates to the preparation of laminated metal articles having a surface metal layer integrally bonded with a backing metal layer.

More specifically this invention relates to the formation of ingots having a plurality of metal slabs disposed in the center thereof and welded to the surrounding metal. The invention includes the preparation of laminated metal sheets from such ingots.

It has heretofore been proposed to cast molten metal entirely around a pair of metal slabs to form an ingot composed of the metal slabs in the center thereof integrally welded with the surrounding cast metal. In my U. S. Patent No. 1,868,749 entitled "Laminated metal and process of making same", issued July 26, 1932, I have described and claimed the process of forming laminated metal sheets by preparing two metal slabs such as stainless steel slabs with finished surfaces, placing said slabs in juxtaposed position with a separating composition therebetween, sealing the slabs together along their adjoining peripheral edges and casting another metal such as mild steel entirely around said slabs to become integrally bonded thereto. I have now provided a process wherein a plurality of pairs of juxtaposed slabs can be used in one casting operation to form a large composite metal ingot from which a plurality of pairs of metal articles can be rolled.

In my co-pending application entitled "Method and apparatus for casting composite metal ingots", Serial No. 753,079 filed November 15, 1934, I have described and claimed a method for suspending the metal slabs in a mold by means of breather pipes welded to the tops of the slabs to permit escape of gases from the space between the slabs. According to my present process, breather pipes can be used in an identical manner as disclosed in my co-pending application. It should be understood, however, that any other means of suspending the slabs in the mold may be used without departing from the principles of this invention.

This process provides for the casting of large composite metal ingots having a plurality of pairs of metal slabs disposed at the core of the ingot. The slabs are joined together either in superimposed or laterally extended relation with separating bars positioned between each pair of slabs along the top or side edges thereof. The separating bars are welded to the top and bottom or sides of the slabs so as to form an integral insert which may be suspended as a unit into a

mold in spaced relation from the walls of the mold. Molten metal having different characteristics from the metal of the slab but having similar characteristics to the metal of the separating bars is then cast entirely around the slabs to form the ingot of this invention which is subjected to a "slabbing down" or rolling operation after cooling to form a pack having the pairs of partially rolled metal slabs in the center thereof. The separating bars being identical with the case metal fuse together with this metal to form an integral mass. The slabbed down pack is next cut into sections each of which have a pair of the partially rolled metal slabs in the center thereof. Each section is then rolled into a sheet form, the marginal edges are clipped off and the laminated metal sheets spring apart.

It is therefore an object of this invention to provide a process for casting large composite metal ingots having a plurality of pairs of metal slabs disposed in the core and integrally bonded with the surrounding metal.

Another object of this invention is to provide a process for preparing a plurality of pairs of laminated metal sheets which process involves only a single casting operation.

A further object of this invention is to provide a method for the mass production of laminated metal sheets wherein a plurality of pairs of said sheets can be formed by a single casting operation.

Other and further objects of this invention will be apparent from the following detailed description of the annexed sheets of drawings which illustrate preferred embodiments of the invention.

On the drawings:

Figure 1 is a front elevational view with parts in cross section, illustrating the manner in which a plurality of pairs of super-imposed metal slabs are suspended in a mold in spaced relation from the walls thereof.

Figure 2 is a cross sectional view taken substantially along the line II—II of Figure 1.

Figure 3 is a cross sectional view of an ingot formed by casting molten metal into the mold illustrated in Figures 1 and 2.

Figure 4 is a plan view of a partially rolled or "slabbed down" pack formed from the ingot shown in Figure 3.

Figure 5 is a view taken substantially along the line V—V of Figure 4.

Figure 6 is a broken cross sectional view of the pack formed after the rolling operation is completed.

5

10

15

20

25

30

35

40

45

50

55

Figure 7 is a broken end elevation of a composite metal sheet formed according to this invention.

Figure 8 is a top plan view illustrating an alternative method for suspending the slabs in a mold.

Figure 9 is a view taken substantially along the line IX—IX of Figure 8.

As shown on the drawings:

10 In Figures 1 and 2 the reference numeral 10 indicates generally a relatively deep mold composed of half sections 11 and 12. The side walls of the mold 10 are provided with laterally extending ears 13 and 14. Bolts 15 and 16 are 15 pivoted in the ears 13 and 14 respectively. A supporting bar 17 of sufficient length to extend across the width of the mold is provided with bifurcated ends through which the bolts 15 and 16 may extend. Wing nuts 18 and 19 are then 20 threaded down on the bolts 15 and 16 to clamp the bar 17 on top of the mold.

The bar 17 is provided with apertures in the central portion thereof of sufficient size to allow the breather pipes 20 and 21 to extend therethrough. Nuts 22 and 23 in threaded engagement with the breather pipes 20 and 21 maintain the bar 17 in proper spaced relation from the bottom of the breather pipes, while nuts 24 and 25 are threaded on the breather pipes over 30 the bar 17 to clamp the bar between the nuts 22 and 24 and 23 and 25.

35 Rectangular metal slabs 26 and 27 are provided with smoothed and cleaned surfaces by a pickling or other cleaning operation and are then placed in juxtaposed relation with a separating material 28 therebetween. The adjoining peripheral edges of the slabs 26 and 27 are next welded together by a weld similar to the weld 29 shown on the lowermost pair of slabs in 40 Figure 2. The weld does not extend across the space occupied by the breather pipes 20 and 21. These breather pipes, on the other hand, are welded to the tops of the slabs 26 and 27 as shown at 30 and 31 to secure the breather pipes 45 to the slabs in communication with the space between the slabs.

A spacer bar 32 is next welded to the bottom of the slabs 26 and 27 around their outside peripheral edges by a weld 33. The bar 32 is provided with holes 34 and 35 extending therethrough. The weld 29 around the adjoining peripheral edges of the slabs 26 and 27 does not extend across these openings 34 and 35.

50 A second pair of metal slabs 36 and 37 welded together in an identical manner with the slabs 26 and 27 and having a separating medium therebetween are welded around their outside peripheral top edges to the bottom of the bar 32 by a weld 38.

60 The bottom of the slabs 36 and 37 is welded to another spacer bar 38 having holes 39 and 40 therethrough by means of a weld 41.

Another pair of metal slabs 42 and 43 secured together by the weld 29 with a separating composition therebetween are welded to the bottom of the bar 38 around their outside top peripheral edges by means of a weld 44.

70 As pointed out above, the weld 29 joining the pairs of metal slabs together in juxtaposed relation does not extend over the openings in the spacer bars 32 and 38 so that the breather pipes 20 and 21 are in communication with the spaces between each pair of slabs.

75 The so-welded together pairs of super-imposed slabs are suspended from the breather pipes 20

and 21 and are held in spaced relation from the walls of the mold 10 by the supporting bar 17.

Molten metal having different characteristics than the metal of the slabs is next poured entirely around the slabs to form the ingot as shown in Figure 3. The spacer bars 32 and 38 and the breather pipes 20 and 21 are preferably formed of metal having the same characteristics as the cast metal so that they will partially melt during the casting operation and fuse with the cast metal to form a homogeneous mass. The cast metal also fuses with the slab metal to become bonded therewith. The ingot 45 shown in Figure 3 therefore is composed of cast metal having a core composed of the plurality of pairs of metal 15 slabs in spaced super-imposed relation. The separating compound between the slabs prevents the same from fusing together during the casting operation.

20 After the ingot 45 has cooled, it is stripped from the mold 10 by removing the half sections 11 and 12 of the mold. The solidified ingot 45 is then "slabbed down" or rolled to form the pack 46 shown in Figures 4 and 5. During this rolling operation, the slabs become more integrally 25 bonded with the cast metal and are rolled out together with the cast metal to form the flat pack. During this rolling operation, the spacer bars 32 and 38 which now have become an integral part of the cast metal are compressed 30 more than the slabs since they are somewhat softer. This feature is very advantageous since it provides depressed portions 47 and 48 (Figure 35 5) between the slabs. The "slabbed down" pack 46 is next cut along the lines X—X (Figure 35 5) to provide three separate packs each of which provide two composite metal sheets as will be hereinafter described. The pack 46 is cut in the center of the depressed portions 47 and 48 and the lines X—X are thereby readily positioned. 40

Each of the portions 49, 50 and 51 of the pack 46 are next rolled down into the sheet or plate pack 52 shown in Figure 6. The marginal edges of the rolled down pack 52 are next clipped off along the lines Z—Z to provide two laminated 45 metal sheets such as the sheet 53 shown in Figure 7. Each sheet 53 is composed of a surface layer 54 of the slab metal integrally bonded with a backing layer 55 of the cast metal.

50 In Figures 8 and 9 I have shown a modified arrangement of the slabs in a mold which is less deep than the mold shown in Figures 1 and 2.

As shown in Figures 8 and 9, an elongated rectangular mold 60 is provided with laterally extending ears 61 and 62 on the sides thereof. The 55 ears 61 and 62 are adapted to receive pivotally mounted bolts 63 and 64 having wing nuts 65 and 66 threaded thereon.

60 A supporting bar 67, of sufficient length to extend across the length of the mold is provided with bifurcated ends 68 and 69 adapted to receive respectively the bolts 63 and 64 therethrough. The wing nuts 65 and 66 clamp the bar 67 on top of the mold 60.

65 Since the bar 67 is necessarily of considerable length, a second supporting bar 70 is provided to reinforce the bar 67 and prevent the same from sagging. The bar 70 extends across the width of the mold resting on the top of the mold walls and is provided with a depressed 70 central portion 71 for receiving the bar 67. The bars 67 and 70 are then clamped together by means of a bolt 72 and a nut 73.

75 The bar 67 is provided, intermediate the ends thereof, with a plurality of holes adapted to re-

ceive breather pipes 74 to 79 inclusive there-through. The bar 67 is clamped to each breather pipe and maintained in spaced relation from the bottom of said pipe by means of nuts 80 and 81 threaded on the breather pipe above and below the bar in a manner identical with that described in connection with Figures 1 and 2.

Pairs of metal slabs 82 and 83; 84 and 85; 86 and 87 are each welded together in juxtaposed relation along their adjoining peripheral edges with a weld 88 to provide a plurality of pairs of metal inserts. The breather pipes 74 and 75 are welded to the tops of the slabs 82 and 83 by welds 89 and 90. The breather pipes 76 and 77 are welded to the tops of the slabs 84 and 85 by welds 91 and 92 while the breather pipes 78 and 79 are welded to the flat tops of the slabs 86 and 87 by welds 93 and 94. The welds 88 joining the slabs together in juxtaposed relation do not extend across the space occupied by the breather pipes so that each pipe is in communication with the space between the slabs. A separating medium is inserted in this space or is coated onto the adjoining surfaces in each pair of slabs.

The respective pairs of slabs are placed in lateral alignment and spacer bars 95 and 96 are inserted between adjoining sides of the slabs. The spacer bar 95 is welded to the slabs 82 and 83 around the outer edges of said slabs by a weld 97. This bar is also welded to the sides of the slabs 84 and 85 which adjoin the slabs 82 and 83 by means of a weld 98.

The opposite sides of the slabs 84 and 85 are welded to the spacer bar 96 by means of a weld 99 while the slabs 86 and 87 are also welded to this spacer bar 96 by a weld 100.

The thus welded together pairs of metal slabs are suspended in the mold 10 from the breather pipes welded along the tops of the slabs by means of the supporting bars 67 and 10. The slabs are in spaced relation from the walls of the mold and molten metal of different characteristics from the metal of the metal slabs is cast entirely around the slabs. The breather pipes and spacer bars are preferably formed of metal having the same characteristics as the cast metal so that they will partially melt down and become integrally fused with the cast metal to form a homogeneous mass. The cast metal also fuses into the exposed surfaces of the metal slabs to become bonded thereto. After the cast metal has solidified, the resulting ingot is stripped from the mold and rolled in an identical manner described in connection with Figures 3 to 7 inclusive. It should be understood that the welds 97 to 100 need not be continuous welds since the spacer bars may be satisfactorily secured to the slabs by a plurality of spaced spot or tack welds. The spacer bars 95 and 96 need not have holes permitting communication of the spaces between the adjoining slabs since each of the slabs are provided with breather pipes for this purpose. The spacer bars 95 and 96, however, could be provided with holes similar to the holes in the spacer bars 32 and 38 and a breather pipe would then only be positioned on each end of a lateral string of the slabs. Thus the breather pipes 74 and 79 could serve all of the slabs since the spaces between the slabs would be in communication with these breather pipes through the holes in the spacer bars. If holes are provided in the spacer bars, the welds 88, of course, would not extend across the holes.

The breather pipes serve a dual purpose of

providing means for suspending the slabs in spaced relation from the walls of the mold and at the same time permitting the escape of gases from the spaces between the slabs during the casting operation. Compressed air or other fluids can be blown through one of the breather pipes and allowed to escape out of the other breather pipe in each pair of the slabs for controlling the cooling rate during the casting operation.

From the above description it is obvious that I have now provided a process wherein a plurality of pairs of metal slabs may be used in a single casting operation for providing a plurality of pairs of metal articles. While three pairs of metal slabs have been illustrated in each instance on the drawings, it should be understood that the invention can be applied to the casting of the molten metal around two or more pairs of slabs. This process greatly reduces manufacturing costs of laminated metal articles since it provides for the mass production of such articles wherein large ingots are prepared by a single casting operation. These ingots having a plurality of pairs of spaced slabs in the core thereof make possible the rolling down of the ingot to form a slabbed down pack with all of the slab metal sealed from the atmosphere. The pack is then clipped between the pairs of slabs without exposing the slab metal to the atmosphere. Each clipped portion can then be further rolled to the finished form without exposing the slabs. The process, therefore, prevents finished surfaces of the slabs from contacting the atmosphere until the rolling operations are completed.

If a single pair of large slabs were inserted in a mold to form the core of a large ingot, this ingot could not be rolled on standard size rolling mills direct to sheet or plate form without shearing into the slab metal to separate portions therefrom of a rollable size. This would expose the slab metal to the atmosphere and might destroy the original prepared surfaces of the slabs. It was therefore necessary heretofore to provide small ingots so that they could be rolled direct to the finished plate, strip or sheet without exposing the slabs to the atmosphere.

The process is applicable to the casting of a ferrous metal about non-ferrous metal slabs as well as to the casting of a ferrous metal such as mild steel around stainless steel slabs.

I am aware that many changes may be made and numerous details of construction may be varied through a wide range without departing from the principles of this invention, and I, therefore, do not purpose limiting the patent granted hereon otherwise than necessitated by the prior art.

I claim as my invention:

1. The method of forming a composite metal ingot, comprising the steps of inserting a separating material between opposed broad faces of paired metal slabs of a plurality of paired metal slabs, sealing certain edges of said pairs by welding corresponding edges of the slabs therein together and leaving other edges unsealed, arranging said pairs of slabs in a common plane with their unsealed edges in opposed relation, coupling said pairs together by means of sealing members disposed between the opposed edges, and casting molten metal of different characteristics than the slab metal entirely about said slabs.

2. The process of forming a composite metal ingot comprising welding together a pair of metal slabs in juxtaposed face to face relation with a separating medium therebetween, capping an

edge of said slabs with a separator bar and welding said bar to said slabs, preparing another pair of slabs welded together in such juxtaposed relation with a separating medium therebetween, 5 welding an edge of said other pair of slabs to said separator bar, supporting said pairs of slabs in an ingot mold, and casting molten metal of different characteristics than the slab metal entirely about said slabs.

10 3. The method of forming a composite metal ingot, comprising the steps of preparing a plurality of paired metal slabs, the slabs in each pair being slightly spaced and in parallelism and there being a weld preventing material within 15 the space between the paired slabs, placing said pairs of slabs in edge to edge relation with an apertured separator bar between such edges and with the apertures in said bar disposed for providing communication with the spaces between 20 the paired slabs, welding said separator bar to the paired slabs on each side thereof, welding a breather pipe to the edge of one of said pairs of slabs and in communication with the space between such pair, suspending all of said slabs from 25 said breather pipe, and casting molten metal of different characteristics than the slab metal entirely about said slabs.

4. The process of forming composite metal ingots, comprising the steps of arranging a plurality of metal slabs in pairs with the slabs of each pair in parallel juxtaposed position, securing the slabs in each pair together about their peripheral edges to provide an envelope between the slabs therein, there being provided a separating 30 composition in each of such envelopes, placing the so formed pairs of slabs in edge to edge relation with a metallic separator bar between such edges, said bars having openings therein in communication with the envelopes of the pairs on 35 each side thereof, welding the separator bars to such edges of the pairs, suspending the thus assembled slabs and pairs in spaced relation from the walls of a mold, and casting a metal having the same characteristics as the separator bars 40 but of different characteristics than the slab metal entirely about said slabs.

5. The process of forming composite metal ingots, comprising the steps of arranging a plurality of metal slabs in pairs with the slabs of each pair in parallel juxtaposed position, securing the slabs in each pair together about their peripheral edges to provide an envelope between the slabs therein, there being provided a separating composition in each of such envelopes, placing 50 the so formed pairs of slabs in edge to edge relation with a metallic separator bar between such edges, said bars having openings therein in communication with the envelopes of the pairs on each side thereof, welding the separator bars to 55 such edges of the pairs, suspending the thus assembled slabs and pairs in spaced relation from the walls of a mold, casting a metal of different characteristics than the slab metal about the insert, allowing the cast metal to cool thereby forming 60 an ingot, rolling the ingot upon a plane parallel to the plane of said slabs thereby forming a flat pack, cutting said pack into lengths containing the metal of one pair of said slabs in each length, further rolling each of said lengths into 65 flat laminated bodies, clipping the marginal edges from said bodies and separating the laminations thereof.

6. The process of forming a plurality of pairs of metal sheets, the process comprising the steps 70 of forming an integral metal insert from a plu-

rality of metal slabs, weld preventing material and metal coupling bars, by arranging said slabs in pairs with the slabs in each pair secured side by side with broad side surfaces in opposed relation and with a quantity of said weld preventing material upon such surfaces, placing said pairs concatenatively in edge to edge relation within a common plane and with said metal coupling bars between said edges of adjacent pairs, securing said bars to such edges, supporting said 10 insert in a mold in spaced relation with the walls thereof, casting a metal of different characteristics than the slab metal entirely around said insert to form an ingot, removing such ingot from the mold, applying pressure to the ingot upon 15 opposite surfaces in parallelism with the plane of said slabs thereby forming a flat pack, separating said pack into a plurality of smaller packs, each of which contains one of said pairs of slabs therein, further compressing each of said smaller 20 packs upon opposite faces parallel to the plane of the slabs therein, clipping the marginal edges from such further compressed packs, and separating such further compressed packs at the plane 25 between the respective slabs therein.

7. The process of forming composite metal sheets, comprising the preparation of a composite metal ingot having a plurality of pairs of juxtaposed metal slabs in the core of the ingot, the pairs being in spaced edge to edge relation and 30 the slabs in each of said pairs having opposed broad sides in spaced relation thereby effecting an interstitial plane therebetween, there being a weld preventing material in such interstices and the interstice within the respective pairs being substantially in a single plane, compressing said ingot upon a plane parallel to the interstitial plane of said pairs whereby to form a flat pack, dividing said pack at the sections between 35 the pairs of metal slabs therein thereby forming a plurality of smaller packs, compressing each of the smaller packs upon its broad surfaces to form laminated sheets of the slabs therein, clipping the marginal edges from the so formed 40 smaller packs and separating the same upon the 45 plane between such sheets.

8. The herein described process of making laminated metal sheets, comprising the steps of forming a plurality of paired metal slabs, the slabs in each pair being disposed with a broad 50 flat side of each in opposed slightly spaced relation with a quantity of weld preventing material therebetween and being joined about their peripheral edges in a manner sealing such space, aligning said pairs within a common plane with 55 an edge of each pair in close proximity with an edge of another pair, joining said pairs together by welding metal bars thereto between such proximate edges, and casting a metal of different characteristics than the slab metal entirely 60 about said slabs.

9. The method of forming a composite metal ingot, comprising the herein described steps of securing flatly together in pairs a plurality of metal slabs with an interstice between the slabs in 65 the respective pairs and with a weld preventing material within such interstices, arranging said pairs coplanary in edge to edge relation with a separator bar between such edges, and joining said edges in such a manner as to obstruct those 70 parts of the interstices coinciding therewith, and casting molten metal of different characteristics than the slab metal entirely about said slabs.